

# UNITED STATES PATENT OFFICE.

ROBERT A. HADFIELD, OF WESTMINSTER, ENGLAND.

## METHOD OF TOUGHENING PROJECTILES.

1,325,987.

Specification of Letters Patent. Patented Dec. 23, 1919.

No Drawing. Application filed April 22, 1914, Serial No. 833,620. Renewed September 18, 1919. Serial No. 324,580.

To all whom it may concern:

Be it known that I, ROBERT ABBOTT HADFIELD, a subject of the King of Great Britain and Ireland, residing at 22 Carlton 5 House Terrace, city of Westminster, England, have invented new and useful Improvements in Methods of Toughening Projectiles, of which the following is a specification.

10 My invention relates to armor piercing projectiles and consists in a method whereby the projectiles are greatly improved as to the toughness of the hardened portions and also as to uniformity both in toughness and 15 hardness.

In the manufacturing of hardened armor piercing projectiles, it has been found that after these have been duly heated, treated and hardened, there is often considerable 20 variation in the hardness at various points and in the character of the hardness. In case of overhardening either in spots or of the whole point, or even when not overhardened, the hardened portion is not so 25 tough as it should be. Consequently when such a projectile, either with or without a cap, strikes an armor plate, it is liable to crack, and such cracking may break up the whole projectile and prevent penetration.

30 I have discovered that if the projectile is then reheated to a substantial degree that is to from 100° C. to 200° C. or even to 250° C. there is a substantial increase in the 35 toughness. This increase is to some extent in proportion to the degree of heating and the higher the temperatures the tougher will be the product, but as it is accompanied by some diminution in the hardness, the heating should not be carried too far that is not 40 above about 250° C. at the highest.

As an example of the treatment; an armor piercing projectile of 12 cm. caliber was hardened in the usual manner and the forward portion of the projectile heated to 45 about 250° C. to within about 3" of the base, it being understood that the projectile was about 12" in length. It was then plunged in the oil bath to its base and maintained there for a short time, then withdrawn and permitted to cool in the air. It

was found that the toughness of this projectile was greatly increased and at the same time its hardness was not substantially diminished. When fitted with a cap, it perforated unbroken a 4" K. C. armor plate. 55

In the tests it was found that hardened projectiles tempered as aforesaid to a temperature about as high as 250° C. all gave a ball hardness of above 600 Brinell scale, but at the same time the toughness was greatly increased, in fact to such an extent in some cases as to permit an 8° bend. This is an extraordinary result for hardened steel, for it will be understood that ordinary hardened steel under the shot test gives practically no 60 bending angle at all. 65

As aforesaid the tempering temperature may be greatly varied and may be carried to as high as 250° C. or thereabout, but in some cases it will be desirable to heat only 70 to about 150° C., whereby the toughness will be decidedly increased without danger of substantially reducing the hardness.

I claim,

1. The method of toughening hardened 75 armor piercing projectiles which consists, after hardening, in heating the projectile to about 150° C., then permitting it to cool.

2. The herein described process of increasing the toughness of hardened projectiles 80 and the like which consists in heating the article from over 100° C. to not over 250° C. and then permitting the article to cool.

3. The herein described method of increasing the toughness and making uniform 85 the hardness of hardened armor piercing projectiles of a substantial size for instance not less than about twelve by three inches, which consists in heating the projectile to a comparatively low degree and above about 90 50° C., then plunging the projectile in an oil bath, then taking it out and permitting it to cool.

In testimony whereof I have signed my name to this specification in the presence of 95 two subscribing witnesses.

ROBERT A. HADFIELD.

Witnesses:

A. F. SASSEEN,  
J. R. MILLWARD.